

## 1

3,720,525

## ELECTROLESS COPPER PLATING SOLUTIONS

## WITH ACCELERATED PLATING RATES

Nathan Feldstein, Kendall Park, and Joel Alan Weiner,  
Cranbury, N.J., assignors to RCA Corporation  
No Drawing. Filed Aug. 16, 1971, Ser. No. 172,300

Int. Cl. C23c 3/02

U.S. CL. 106—1

4 Claims

## ABSTRACT OF THE DISCLOSURE

The rate of plating copper onto an active metallic surface of a substrate from an electroless copper plating solution is enhanced by adding to the plating solution an ionic compound consisting of either an acetate, a nitrate, an oxalate, a lactate, a chloride, a tartrate, a formate, a phthalate, a tungstate, a molybdate, a chlorate, a perchlorate, a citrate, a malonate, or mixtures thereof.

## BACKGROUND OF THE INVENTION

This invention relates generally to electroless plating solutions, and more particularly to improved electroless copper plating solutions with accelerated plating rates.

The process of electroless plating is used in the manufacture of printed and hybrid circuits in the electronic industry. Generally, a relatively thin film of copper is electrolessly deposited upon a specially prepared surface of a dielectric substrate, and the deposited film is subsequently electroplated with copper to a desired thickness. Thus, the substrate may be electrolessly plated initially with a copper film of about 0.01 mil, for example, and then electroplated with copper to a thickness of between 1-2 mils. Since the rate of the electroless deposition of copper onto a substrate is relatively slow, it is advantageous to enhance the deposition rate, thereby increasing the rate of production and consequently reducing the cost per unit of construction.

It has been proposed to accelerate the rate of the electroless deposition of copper by increasing the temperature of the plating solution, but this procedure is not always desirable or practical because increased temperatures may either reduce the stability of some plating solutions and/or adversely affect certain materials that are temperature sensitive, such as photoresists, that may already be on the substrate.

The improved copper plating solutions of the present invention may be used at normal room temperatures and yet provide enhanced rates of deposition of copper in comparison with the electroless copper plating solutions of the prior art.

## SUMMARY OF THE INVENTION

Each of the improved electroless copper plating solutions with accelerated plating rates comprises the combination of an electroless copper plating solution with an accelerator that is a compound consisting of either an acetate, a nitrate, an oxalate, a lactate, a chloride, a tartrate, a formate, a phthalate, a tungstate, a molybdate, a chlorate, a perchlorate, a citrate, a malonate, or mixtures thereof. A preferred embodiment of an improved accelerated electroless plating solution comprises one wherein a cupric ion complex is the reaction product of an ethyleneaminoacetic acid, preferably propylenediaminetetraacetic acid, and a cupric compound. The propylenediaminetetraacetic acid, (hereinafter referred to as PDTA), should contain no more than 10%, by weight, of nitrilotriacetic acid (hereinafter referred to as NTA),

## 2

a by-product normally produced in the commercial manufacture of PDTA and usually combined therewith.

## DESCRIPTION OF THE PREFERRED EMBODIMENTS

In accordance with the present invention, the rate of deposition of copper from an electroless copper plating solution is enhanced by adding certain ionic accelerators to the plating solution. These ionic accelerators are relatively inexpensive salts that form an improved combination with electroless copper plating solutions to enhance the rate of deposition of copper therefrom without the necessity of increasing the operating temperature of the plating solution. Also, these accelerators are not consumed during the plating process.

The ionic accelerators for combination with electroless plating solutions to provide improved solutions are soluble salts of an acetate, a nitrate, an oxalate, a lactate, a chloride, a tartrate, a formate, a phthalate, a tungstate, a molybdate, a chlorate, a perchlorate, a citrate, a malonate, or mixtures thereof. While these ionic accelerators may have any cation, as for example, sodium, potassium, or ammonium cations, the sodium salts of the accelerators are preferred because they are usually the least expensive. These novel ionic accelerators when used in combination with prior-art electroless plating solutions markedly accelerate the plating rate. The improved electroless plating solutions may also contain wetting agents, buffers, brighteners, and stabilizers, well known in the art.

Most electroless copper plating solutions are similar in their essential composition. They generally contain metallic cations as the source of metal to be deposited, a reducing agent, a chelating (or complexing) agent to prevent precipitation of any insoluble metallic salts, and pH regulators to maintain the solution between a pH of 10 and 14. A preferred electroless copper plating solution for combination with one or more of the accelerators of the present invention to enhance the rate of deposition of copper therefrom is as follows:

## ELECTROLESS COPPER PLATING SOLUTION I

15.0 g./l. CuSO<sub>4</sub>·5H<sub>2</sub>O  
53.0 ml./l. 40% active solution of PDTA (as Na<sub>4</sub> salt)  
15.0 ml./l. 37% H<sub>2</sub>CO  
4.0 g./l. NaOH  
4×10<sup>-3</sup> g./l. NaCN  
4.1×10<sup>-3</sup> g./l. TMN ("Tergitol" a non-ionic surfactant of Union Carbide Co.—a trimethyl monylether of polyethylene glycol containing 6 moles of ethylene oxide)

In the electroless copper plating Solution I, the copper sulfate is a source of metallic copper, providing cupric ions. The formaldehyde provides the reducing power for the bath. The PDTA is the complexing agent used to complex the copper ions to prevent the precipitation of copper as a hydroxide. The sodium hydroxide adjusts the pH of the solution to the proper alkalinity. The cyanide stabilizes the solution; and the "Tergitol" is a wetting agent that also functions, in combination with the cyanide, to brighten the deposited copper. The quantities of the ingredients of the Solution I, and other solutions described herein, are not critical and may vary within limits well known in the art. The PDTA used as the chelating agent in Solution I is generally not a pure compound because the pure product is relatively expensive. Commercial PDTA is usually sold with nitrilotriacetic acid (NTA) as a combined by-product, but the NTA should not be present in a quantity of more than 10%,

by weight, of the product. NTA also functions as a chelating agent.

PDTA is an ethyleneaminoacetic acid. Other ethyleneaminoacetic acids that may be substituted for the PDTA in Solution I in suitable amounts are ethylenediaminetetraacetic acid, diethylenetriaminepentaacetic acid, and 1,2-cyclohexylenediaminetetraacetic acid.

The novel ionic accelerators of the following Table I were combined with the electroless plating Solution I and the increase in the plating rate was noted:

TABLE I.—IONIC ACCELERATORS IN SOLUTION OF SOLUTION I

| Ionic accelerator                                                                  | Molar-<br>ity in<br>Solu-<br>tion I | Mg. of<br>copper<br>plated<br>out | Percent<br>increase<br>in plat-<br>ing rate | 15 |
|------------------------------------------------------------------------------------|-------------------------------------|-----------------------------------|---------------------------------------------|----|
| None (control)                                                                     |                                     | 8                                 | -----                                       |    |
| NaCH <sub>3</sub> CO <sub>2</sub> (sodium acetate)                                 | 1                                   | 13.0                              | 62                                          |    |
| NaNO <sub>3</sub> (sodium nitrate)                                                 | 1.5                                 | 12.8                              | 60                                          |    |
| K <sub>2</sub> C <sub>8</sub> O <sub>4</sub> ·H <sub>2</sub> O (potassium oxalate) | 2%                                  | 15.4                              | 93                                          | 20 |
| NaC <sub>3</sub> H <sub>5</sub> O <sub>3</sub> (sodium lactate)                    | 2                                   | 13.5                              | 69                                          |    |
| NaCl (sodium chloride)                                                             | 4                                   | 11.9                              | 49                                          |    |
| NaKC <sub>4</sub> H <sub>4</sub> O <sub>6</sub> (sodium potassium tartrate)        | 1                                   | 12.7                              | 59                                          |    |
| NaHCO <sub>2</sub> (sodium formate)                                                | 2                                   | 14.4                              | 79                                          |    |
| NaKC <sub>8</sub> H <sub>6</sub> O <sub>4</sub> (sodium potassium phtha-<br>late)  | 1                                   | 14.7                              | 84                                          |    |
| Na <sub>2</sub> WO <sub>4</sub> (sodium tungstate)                                 | 1                                   | 13.0                              | 62                                          | 25 |
| Na <sub>2</sub> MoO <sub>4</sub> (sodium molybdate)                                | 1                                   | 12.9                              | 61                                          |    |
| NaClO <sub>3</sub> (sodium chlorate)                                               | 1                                   | 12.8                              | 60                                          |    |
| NaClO <sub>4</sub> (sodium perchlorate)                                            | 1                                   | 12.1                              | 51                                          |    |
| Na <sub>3</sub> C <sub>6</sub> H <sub>5</sub> O <sub>7</sub> (sodium citrate)      | 1                                   | 10.7                              | 34                                          |    |
| Na <sub>2</sub> C <sub>4</sub> H <sub>2</sub> O <sub>4</sub> (sodium malonate)     | 1                                   | 10.0                              | 25                                          |    |

In each of the examples of the combinations of the 30 ionic accelerators and Solution I given in Table I, the Solution I was first saturated with nitrogen to remove any dissolved oxygen. Also, in each example, copper was allowed to plate out from the solution onto an active metallic surface of a substrate of a 2-inch square ceramic wafer at a temperature of 25° C. for a period of 10 minutes. The amount of an ionic accelerator that may be combined with an electroless plating solution is determined by the solubility of the accelerator in the solution. For practical purposes, the amount of ionic accelerator used should form at least a 0.1 molar solution with the electroless copper solution. Actually, the ionic accelerator may be added to the electroless plating solution until the solution is saturated. The percentage of 45 increase in the rate of deposition of copper from the solution is substantially proportional to the amount of the ionic accelerator used. For example, successive applications of sodium acetate in concentrations on the order of 0.5, 1.0, and 1.5 moles to the electroless copper plating Solution I accelerated the plating rates 25%, 62%, and 93%, respectively.

Any clean active metallic surface that is not adversely affected by alkaline aqueous solutions can be plated with the copper plating Solution I merely by bringing the 55 active metallic surface into contact with the plating solution, or by suitable pretreatment known in the art. Typical active metallic surfaces that can be copper plated by the Solution I are, for example, clean surfaces of iron, cobalt, gold, silver, palladium, platinum, rhodium, 60 copper, and alloys thereof.

Non-metallic surfaces can be copper plated by the Solution I but the non-metallic surfaces must first be provided with a catalytic metal to accept the copper plating. It is preferable to first roughen the non-metallic surface either by chemical or mechanical means, such as by chemical etching or by sand blasting. The non-metallic surface is next treated with a sensitizing stannous chloride solution, followed by washing with water and then treating with an activating solution of a silver, 70 gold, or palladium salt that will provide a catalytic film of the particular metal used. Thus, the non-metallic surface is provided with an active metallic surface on which the copper can be plated when brought into contact with an electroless copper plating solution.

In the following electroless copper plating Solutions II–VIII, ionic accelerator salts were added in amounts to form one molar concentrations of the solutions, and the percentages of increase in the plating rates were observed as indicated in the corresponding Tables II–VIII, respectively. The conditions of plating in the following examples were the same for each example, and were the same as those described for the plating of copper on a 2-inch square ceramic substrate from the electroless plating Solution I (i.e. 25° C., 10 minutes).

ELECTRODES COPPER PLATING  
SOLUTION II

|                                                  |
|--------------------------------------------------|
| 15.0 gr./l. CuSO <sub>4</sub> ·5H <sub>2</sub> O |
| 53.0 ml./l. PDTA Na <sub>4</sub> (40% solution)  |
| 4.0 gr./l. NaOH                                  |
| 15.0 ml./l. H <sub>2</sub> CO (37% solution)     |
| 0.004 gr./l. NaCN                                |

TABLE II

| Ionic accelerator added           | Weight of<br>Cu depos-<br>ited (mg.) | Percent<br>increase in<br>plating rate |
|-----------------------------------|--------------------------------------|----------------------------------------|
| None                              | 19.9                                 | -----                                  |
| NaCH <sub>3</sub> CO <sub>2</sub> | 35.0                                 | 75                                     |
| KNO <sub>3</sub>                  | 36.3                                 | 81                                     |

ELECTROLESS COPPER PLATING  
SOLUTION III

|                                                  |
|--------------------------------------------------|
| 15.0 gr./l. CuSO <sub>4</sub> ·5H <sub>2</sub> O |
| 53.0 ml./l. PDTA Na <sub>4</sub> (40% solution)  |
| 4.0 gr./l. NaOH                                  |
| 15.0 ml./l. H <sub>2</sub> CO (37% solution)     |
| 0.00014 gr./l. "Tergitol" TMN                    |

TABLE III

| Ionic accelerator added           | Weight of<br>Cu depos-<br>ited (mg.) | Percent<br>increase in<br>plating rate |
|-----------------------------------|--------------------------------------|----------------------------------------|
| None                              | 24.7                                 | -----                                  |
| NaCH <sub>3</sub> CO <sub>2</sub> | 52.4                                 | 110                                    |
| KNO <sub>3</sub>                  | 48.7                                 | 95                                     |

ELECTROLESS COPPER PLATING  
SOLUTION IV

|                                                  |
|--------------------------------------------------|
| 15.0 gr./l. CuSO <sub>4</sub> ·5H <sub>2</sub> O |
| 53.0 ml./l. PDTA Na <sub>4</sub> (40% solution)  |
| 4.0 gr./l. NaOH                                  |
| 15.0 ml./l. H <sub>2</sub> CO (37% solution)     |
| 0.00014 gr./l. "Tergitol" TMN                    |

TABLE IV

| Ionic accelerator added           | Weight of<br>Cu depos-<br>ited (mg.) | Percent<br>increase in<br>plating rate |
|-----------------------------------|--------------------------------------|----------------------------------------|
| None                              | 46.0                                 | -----                                  |
| NaCH <sub>3</sub> CO <sub>2</sub> | 56.6                                 | 23                                     |
| KNO <sub>3</sub>                  | 55.8                                 | 21                                     |

ELECTROLESS COPPER PLATING  
SOLUTION V

|                                                                                    |
|------------------------------------------------------------------------------------|
| 7.5 gr./l. CuSO <sub>4</sub> ·5H <sub>2</sub> O                                    |
| 15.0 gr./l. sodium salt of ethylenediaminetetraacetic acid (EDTA Na <sub>4</sub> ) |
| 20.0 gr./l. NaOH                                                                   |
| 40.0 ml./l. H <sub>2</sub> CO (37% solution)                                       |
| 0.1 gr./l. NaCN                                                                    |

TABLE V

| Ionic accelerator added           | Weight of<br>Cu depos-<br>ited (mg.) | Percent<br>increase in<br>plating rate |
|-----------------------------------|--------------------------------------|----------------------------------------|
| None                              | 10.2                                 | -----                                  |
| NaCH <sub>3</sub> CO <sub>2</sub> | 15.0                                 | 47                                     |
| KNO <sub>3</sub>                  | 14.3                                 | 40                                     |

ELECTROLESS COPPER PLATING  
SOLUTION VI

15.0 gr./l. Cu(NO<sub>3</sub>)<sub>2</sub>·3H<sub>2</sub>O  
30.0 gr./l. NaKC<sub>4</sub>H<sub>4</sub>O<sub>6</sub>·4H<sub>2</sub>O  
10.0 gr./l. NaHCO<sub>3</sub>  
20.0 gr./l. NaOH  
100.0 ml./l. H<sub>2</sub>CO (37% solution)

TABLE VI

| Ionic accelerator added           | Weight of Cu deposited (mg.) | Percent increase in plating rate |
|-----------------------------------|------------------------------|----------------------------------|
| None                              | 16.6                         | -----                            |
| NaCH <sub>3</sub> CO <sub>2</sub> | 19.3                         | 16                               |
| KNO <sub>3</sub>                  | 19.4                         | 17                               |

ELECTROLESS COPPER PLATING  
SOLUTION VII

15.0 gr./l. Cu(NO<sub>3</sub>)<sub>2</sub>·3H<sub>2</sub>O  
30.0 gr./l. NaKC<sub>4</sub>H<sub>4</sub>O<sub>6</sub>·4H<sub>2</sub>O  
10.0 gr./l. NaHCO<sub>3</sub>  
20.0 gr./l. NaOH  
100.0 ml./l. H<sub>2</sub>CO (37% solution)  
0.02 gr./l. NaCN

TABLE VII

| Ionic accelerator added           | Weight of Cu deposited (mg.) | Percent increase in plating rate |
|-----------------------------------|------------------------------|----------------------------------|
| None                              | 15.3                         | -----                            |
| NaCH <sub>3</sub> CO <sub>2</sub> | 18.8                         | 23                               |
| KNO <sub>3</sub>                  | 17.8                         | 16                               |

ELECTROLESS COPPER PLATING  
SOLUTION VIII

5.0 gr./l. CuSO<sub>4</sub>·5H<sub>2</sub>O  
5.0 gr./l. NaOH  
30.0 ml./l. H<sub>2</sub>CO (37% solution)  
25.0 gr./l. Na<sub>3</sub>C<sub>6</sub>H<sub>5</sub>O<sub>7</sub>·2H<sub>2</sub>O

TABLE VIII

| Ionic accelerator added           | Weight of Cu deposited (mg.) | Percent increase in plating rate |
|-----------------------------------|------------------------------|----------------------------------|
| None                              | 10.7                         | -----                            |
| NaHCO <sub>3</sub>                | 17.9                         | 67                               |
| NaCH <sub>3</sub> CO <sub>2</sub> | 17.5                         | 63                               |
| KNO <sub>3</sub>                  | 19.5                         | 82                               |

The Solutions V, VI, and VIII, without any accelerating compounds, are described in detail in U.S. Patents 3,095,309, 2,874,072, and 3,259,559, respectively.

The electroless plating solutions described herein were premixed, but the reducing agent (formaldehyde) was separated from the oxidizing agent (copper salt) for storage purposes. This precaution was taken because of the thermodynamic metastability of electroless copper plating solutions. Where a cyanide was used, it was premixed with the formaldehyde and kept separated from the sodium hydroxide until needed to prevent the rapid deterioration of the solutions.

Several different substrate materials, such as laminated plastic boards commonly used in the manufacture of printed circuits, were also copper plated with good results. The 2-inch square alumina ceramic wafers (#516 Plain-American Lava Corporation), having a thickness of 0.025" and a surface roughness of 40 micro-inches, however, were used to obtain the data shown in Tables I-VIII because of their uniformity of surface roughness. It should be noted that the data in Tables I-VIII would ordinarily vary with variations in the surface roughness of the substrates used.

The substrates of the experiments were spun dried and weighed before and after the copper deposition cycle. In

all of the experiments, the volume of each of the electroless plating solutions was maintained at 200 ml., and the copper plating was carried out without any external agitation. Also, in all of the experimental data recorded

- 5 in Tables I-VIII, only a single component, the ionic accelerator salt, was varied while the other components were held constant. It has also been observed that in those electroless copper plating solutions from which the initial deposits of copper were dull in color, the addition 10 of a cyanide and a non-ionic surfactant to the solutions increased the brightness of the copper deposited. Although the mechanism by which the ionic accelerator salts enhance the plating rate of electroless copper plating solution is not understood, the combination of these 15 ionic accelerators with the electroless plating solutions provide improved solutions that markedly accelerate the plating rate of copper without substantially altering the quality of the copper deposited. When more than one of the ionic accelerators were combined with an electroless copper 20 plating solution, the percentage of plating rate increase was at least as great as it would be if the ionic accelerator providing the greatest rate increase were added alone.

While the improved electroless copper plating solutions may be used satisfactorily at room temperature, their 25 use is not limited thereto. The improved solutions also exhibit accelerated copper plating rates at elevated temperatures.

We claim:

1. In an electroless copper plating solution which comprises a source of cupric ion, a reducing agent for cupric ion and a pH regulator, the improvement consisting of an additional ingredient which is a plating accelerator in an amount to provide a concentration between 0.1 molar and a saturated solution thereof, where said additional 35 ingredient is a compound selected from the group consisting of sodium or potassium or ammonium nitrate, oxalate, lactate, chloride, formate, phthalate, tungstate, molybdate, chlorate, perchlorate, malonate, and mixtures thereof.
2. A solution according to claim 1 in which said source of cupric ion is a complex which is the reaction product resulting from mixing solutions of an ethyleneaminoacetic acid and a soluble cupric compound.
3. A solution according to claim 1 in which said source 45 of cupric ion is a complex which is the reaction product resulting from mixing solutions of propylenediaminetetraacetic acid and a soluble cupric compound.
4. In an electroless copper plating solution which comprises a source of cupric ion, a reducing agent for cupric ion, a complexing agent for cupric ion and a pH regulator, the improvement consisting of an additional ingredient which is a plating accelerator in an amount to provide a concentration between 0.5 molar and a saturated solution thereof, where said additional ingredient is 50 sodium, or potassium or ammonium acetate.

## References Cited

## UNITED STATES PATENTS

|    |           |         |                       |       |
|----|-----------|---------|-----------------------|-------|
| 60 | 3,310,430 | 3/1967  | Schneble et al. ----- | 106-1 |
|    | 3,370,974 | 2/1968  | Hepper -----          | 106-1 |
|    | 3,377,174 | 4/1968  | Torigai et al. -----  | 106-1 |
|    | 3,515,563 | 6/1970  | Hodoley et al. -----  | 106-1 |
| 65 | 3,615,733 | 10/1971 | Shipley et al. -----  | 106-1 |
|    | 3,663,242 | 5/1972  | Gulla et al. -----    | 106-1 |

LORENZO B. HAYES, Primary Examiner

U.S. Cl. X.R.